

Feb. 27, 1940.

J. FLEISCHER ET AL  
PREPARATION OF CELLULOSE DERIVATIVES

2,191,525

Filed May 5, 1937



INVENTORS  
JOSEPH FLEISCHER  
WILLIAM A. BAILEY JR.

BY  
*Edwards, Bowes & Pool*  
ATTORNEYS

## UNITED STATES PATENT OFFICE

2,191,525

## PREPARATION OF CELLULOSE DERIVATIVES

Joseph Fleischer, Clifton Terrace, Ill., and William A. Bailey, Jr., Baltimore, Md., assignors to The Cellulose Research Corporation, East Alton, Ill., a corporation of Delaware

Application May 5, 1937, Serial No. 140,820

7 Claims. (Cl. 260—227)

This invention relates to the manufacture of cellulose acetate and more particularly to the dehydration of cellulose prior to the acetylation thereof.

5 An object of this invention is to provide an acetylation process by means of which commercially valuable cellulose acetate may be produced from cellulosic materials such as purified wood pulp.

10 Another object of this invention is to provide an economical process for the dehydration and subsequent acetylation of cellulose.

A further object of this invention is to provide a process for the dehydration of cellulose 15 by a distillation method whereby moisture can be removed without substantial shrinkage of the fibers and whereby resinous impurities may be extracted from the fibers at the same time.

Another object of this invention is to provide 20 a process for dehydrating cellulose by distillation whereby the dehydrated cellulose may be directly acetylated without the customary pre-treatment with acetic acid.

Another object of this invention is to provide 25 a process for the dehydration, prior to acetylation, of cellulose, initially in a water-saturated condition, wherein the moisture is removed by distillation while the direct vaporization of moisture from the fibers is avoided.

30 In the commercial processes for the manufacture of cellulose acetate, the initial treatment has consisted in drying purified cotton linters, which have almost exclusively constituted the starting cellulose material for this purpose, to a moisture content of about 2% to 5%, usually by 35 means of hot air. The removal of moisture is essential since it would otherwise react with and cause a wasteful usage of the acetylating reagent, usually acetic anhydride, which is the most expensive raw material employed in the process.

40 However, the drying as conventionally carried out is accompanied by disadvantageous effects, which have been recognized and referred to in the art as loss of reactivity of the fibers. This 45 loss of reactivity is undoubtedly connected with and probably largely due to the shrinkage of the fibers on drying, which is so extensive as to cause a considerable decrease in their cross-sectional area and the almost complete closure 50 of the lumina. The shrinkage in external dimensions is evidently accompanied by a large decrease in the area of cellulose membranes within the fibers which is available for contact with treating liquids such as an acetylation mixture. It has therefore been general practice in

the commercial acetylation processes of the prior art to provide a pretreatment of the dried linters with acetic acid, with or without a catalyst, for an extended period, usually of 4 to 6 hours' duration, at an elevated temperature prior to the 5 addition of the active acetylating reagent, in order to improve this condition.

The lengthening of the acetylation process is an obvious disadvantage of the above procedure. Furthermore, it is properly operative for purified 10 cotton linters only when the evaporation of moisture has been carried out at temperatures below about 70° C. and the moisture content has not been reduced below about 2% or 3%. It should be noted that the state of swelling of the fibers 15 and of the availability of the cellulose to treating liquids is not restored to the conditions originally existing in the water-saturated fibers, which can, for example, be maintained when the water is removed by displacement with acetic 20 acid.

Numerous attempts have been made in the past to substitute purified wood pulp for cotton linters in the manufacture of cellulose acetate, but the acetate solutions obtained therewith by processes 25 which have proven suitable for the conversion of linters have been colored and hazy and yielded products of inferior physical properties even when the starting material consisted of wood pulp having analytical constants approaching 30 those of purified linters. An important reason for this contrast is that the wood fibers, being much more swollen in water-saturated condition than the cotton linters due to the removal of impurities from throughout the cell wall and to the 35 swelling action of concentrated alkaline solutions, undergo greater shrinkage and loss of reactivity on being dried. The conventional pre-treatment with acetic acid therefore does not serve to restore conditions for contact of the 40 cellulose with the acetylating reagents as adequately as in the case of cotton linters.

Apparatus which is suitable for carrying out the process of this invention, as illustrated diagrammatically in the drawing, may consist of a 45 distillation vessel 1, fractionating column 5, condenser 12, receiver 14, and the necessary connections and auxiliary tanks, all parts in contact with liquid or gaseous acetic acid being constructed of material, such as stainless steel, 50 which is resistant to attack by acetic acid. The vessel 1 is provided with a suitable heating jacket, not shown in the figure, perforated metal trays 2, distributing plate 3, and door 4 for charging and discharging the cellulose. Fractionat- 55

ing column 5 may be the plate or packed column type. Thermometers 8 are provided at various points in the apparatus to enable control of the distillation. Condenser 12 is provided with a cooling coil or jacket (not shown in the figure), and likewise receiver 14 if necessary, as when the distillation is carried out at reduced pressure. Tanks 6 and 18 serve as storage tanks for glacial acetic acid and solvent, respectively. Vessels 6, 14, and 18 are provided with calibrated gauge glasses not shown in the figure, to enable the measurement of the volume of contained liquid.

In carrying out the process, a charge of cellulose of known water content is placed on the tray 2 and the door 4 is closed and hermetically sealed. The required volume of glacial acetic acid is measured into the lower part of column 5 from tank 6 through connecting pipe 7, and becomes associated with the cellulose charge after passing through distributing plate 3. The necessary volume of fresh solvent is measured into the bottom space below the trays 2, of vessel 1 from tank 18 through connecting pipe 9 or solvent recovered from a previous distillation is obtained from receiver 14 by means of pipe 16. Heat is supplied to the jacket of vessel 1 at a rate such that the temperature readings of thermometers 8 follow a predetermined schedule. Vapor containing solvent, water, and acetic acid passes to column 5 where it is subjected to fractional condensation so that the vapor passing to condenser 12 through pipe 11 contains mainly solvent and water vapor and only a slight amount of acetic acid. The condensate passes from condenser 12 through pipe 13 into receiver 14, when it separates into a water layer and a solvent layer. The completion of the distillation is indicated when the proper volume of water and solvent layers has collected in receiver 14. The cellulose may then be transferred to the acetylator, after cooling to room temperature if desired. The aqueous layer which has collected in receiver 14 may be removed through pipe 17 and discarded or subjected to treatment for the recovery of dissolved solvent as conditions warrant.

If desired, the distillation may be carried out in whole or in part at a pressure below atmospheric, vacuum line 15, supplied with suitable gauges, being provided for this purpose. When a vacuum distillation is employed, receiver 14 is cooled by means of a jacket or suitable cooling coil.

The arrangement of pipes 16 and 17 in receiver 14, illustrated in Figure 1, is that suitable for use with a solvent having a lower density than water, and would be reversed for use with a solvent which is denser than water.

In this manner cellulose fibers having suitable purity can be converted to a substantially anhydrous condition in a form in which they are readily reactive toward acetylating mixtures by initially supplying the fibers saturated with water, adding acetic acid to the fibers, and removing the water by distillation with the vapor of an organic solvent which is immiscible with water and has other properties as specified hereinafter. By this means the moisture in the fibers is caused to diffuse into the surrounding liquid, from which it is removed by vaporization, while the fibers retain their original swollen condition by virtue of the acetic acid which, during the treatment, replaces the water originally present in the fibers. The organic solvent may be added to the mixture of cellulose and acetic acid as liquid and then caused

to vaporize by the application of heat or may be applied to the mixture directly as vapor.

The starting cellulosic material may consist of purified cellulose from any source, such as wood fibers or cotton linters. For the preparation of cellulose acetate of high quality, the purity and properties of the cellulose fibers should be such that they are convertible, starting from the water-saturated condition and after displacement of the water by acetic acid, by treatment with an acetylating mixture to a useful cellulose acetate solution having low color and haze. Examples of suitable celluloses for this invention are described in the copending applications of Lionel Goff, S. N. 113,155, filed November 28, 1936; of Lionel E. Goff et al., S. N. 81,845, filed May 26, 1936; and of Lyle Sheldon et al., S. N. 126,362, filed February 18, 1937. A procedure for testing the suitability of a cellulose sample for the purpose of this invention will be found at the end of the specification.

The moisture content of the cellulose for treatment by the process of this invention should be between  $\frac{1}{2}$  and 3 times the oven-dry weight of cellulose. A desirable upper limit of moisture content can be generally stated as the residue which cannot be readily removed by pressing the water-wet fibers. The lower limits, the least amount which yields a product having a satisfactory reactivity toward acetylating reagents, will generally be found to be somewhat above the fiber-saturation point.

The amount of acetic acid to be added to the water-wet cellulose may be varied according to conditions from 3 to 7 times the weight of oven-dry material. The amount added must be at least sufficient so that proportionate amounts of the liquids present in the mixture before distillation form a homogeneous liquid phase at distillation temperature. Since the amounts of the other liquids are generally fixed, as will be pointed out hereinafter, the lower limit of the amount of acetic acid which may be used is determined by the above criterion of total miscibility.

The organic solvent to be used in the process of this invention is a liquid or mixture of liquids which is immiscible with water, totally miscible with acetic acid, has a normal boiling point preferably between 75° and 105° C., and forms with water a mixture having an azeotropic boiling point below that which tends to degrade the cellulose. Hydrocarbons, esters, and ethers having the specified properties, for example, benzene, propyl acetate and a mixture of isopropyl ether and isopropyl acetate are particularly suitable, while halogenated derivatives such as ethylene chloride, having a tendency to hydrolyze and liberate halogen acid in the presence of water and therefore exert deleterious action on cellulose, are less desirable. The total amount of solvent added must be sufficient so that on substantially complete removal of same by distillation, substantially all the moisture will also have been evaporated, leaving a residue consisting of cellulose fibers saturated with acetic acid. The minimum quantity of solvent corresponds in general with the amount which would have to be added to the amount of water which is contained in the cellulose to give the azeotropic mixture of the solvent and water. The minimum parts by weight of solvent to be used per part of water in the cellulose are as follows for a number of typical solvents: benzene, 10.4; n-propyl acetate, 6.0; isopropyl acetate, 9.0; and ethyl acetate, 11.2. The composition of azeotropic mixtures can be found

in reference books or readily determined by experiment. If a solvent which meets the above requirements is used in the concentration of the dilute acetic acid solutions resulting from the acetylation process, it will generally be most convenient to utilize the same solvent in the dehydration treatment of this invention. Preferably, an excess of solvent is used, up to 30% or 40% over the amount required to form the azeotropic mixture.

The dehydration may be carried out in any convenient distillation apparatus, such as may be well known in the art, the portions which come into contact with acetic acid being constructed of material resistant to acetic acid. When heat is supplied to the mixture containing cellulose, water, acetic acid, and solvent, for example, by means of a suitable jacket, vapor which consists of solvent, water, and a small proportion of acetic acid, is evolved from the liquid phase. By means of an appropriate fractionating column, substantially only water and solvent vapor are passed to the condenser. The distillate which collects separates into a solvent layer and a water layer; the former is suitable for re-use in the process while the latter may be discarded or treated for recovery of dissolved solvent, as conditions warrant. The distillation is continued until the moisture content of the cellulose is 2% or less. Small losses of acetic acid from the cellulose by distillation are of no special consequence nor is it disadvantageous to have small amounts of solvent remain in the cellulose after the treatment. By measuring the volumes of the layers of distillate which collect, it is possible to follow the course of the dehydration process and control it accordingly.

The distillation may be carried out at atmospheric or reduced pressure and at corresponding temperatures, care being taken to maintain the temperature of the cellulose below the order of 105° C. to avoid the degradation thereof. The time of distillation may be of the order of 4 hours or less depending on the apparatus, amount and type of cellulose being treated, and the temperature and pressure of distillation. However, when the optimum conditions have been determined for a given installation and material, they are maintained constant with successive lots. It may be advantageous at times to conduct the initial part of the distillation at atmospheric pressure and complete the process at reduced pressure. Other variations are possible, for example, instead of adding all the solvent required before the start of the distillation, portions may be added throughout the treatment.

We have further discovered that the purity of the cellulose may be enhanced by the process of this invention through effecting the extraction of resinous and fatty impurities during the distillation. This may be accomplished by placing the cellulose on a perforated tray or within a metal-wire basket in the distillation vessel beneath which liquid may collect during the distillation. Arrangements are preferably such that the reflux from the fractionating column is returned to the upper surface of the mass of cellulose. This returned liquid percolates through the mass of cellulose, extracting resinous and fatty impurities, which remain as a deposit on the bottom of the distillation vessel at the end of the treatment.

The dehydration and extraction may likewise be carried out by a procedure in which the water-saturated cellulose containing the proper quantity of acetic acid is placed on a perforated tray

or trays and the organic solvent is initially contained in the lower portion of the distillation vessel, out of contact with the cellulose. Solvent vapor, which is generated on the application of heat, causes the removal of moisture from the cellulose, and the reflux liquid accomplishes the extraction of resinous and fatty impurities from the fibers, as described above.

Another important advantage of the process of this invention is that it is readily applicable to the dehydration of cellulose fibers which have been subjected to a thorough mechanical beating operation in the presence of water to increase the surface available to liquids. When such beaten fibers are dried by means of hot air or vacuum drying methods, the beneficial effects of the beating treatment are offset by the increased shrinkage and bonding of the fibers and fiber elements, such as occur during the manufacture of paper, and for that reason, it has been desirable to avoid any beating of cellulose fibers intended for use in the conventional acetylation processes. Likewise, it is not practical to dehydrate well-beaten fibers by displacement with a liquid column of acetic acid due to the greatly increased pressures required compared to a similar process applied to unbeaten fibers.

In order more particularly to describe the present invention, there follows the description of typical embodiments of the invention. It will be understood that the various features set forth in connection with these embodiments are by way of illustration only and may be considerably varied within the scope of the present invention.

#### Example A

Purified wood cellulose, for example, that prepared from unbleached spruce sulfite pulp by the process described in the copending application of Lionel Goff, S. N. 113,155, containing, for example, 98.6% alpha cellulose, 2.6% of soda soluble material, and having a cuprammonium viscosity of 14.8 centipoises (see definitions at end of specification), may constitute the starting cellulosic material. The pulp, containing 1.75 times its weight of water is placed in a distillation vessel and treated with 7 times its weight of acetic acid and 24 times its weight of benzene, as described above.

Heat is applied to the distillation vessel jacket to raise the temperature of the cellulose to 50° C. and the distillation is then started by applying vacuum to the system. The temperature is gradually raised during a 2 hour period to 80° C. and the pressure reduced to the order of half an atmosphere, while the distillation is continued. Finally, with the temperature at 80° C., the pressure is reduced to one-third an atmosphere for a short time in order to complete the treatment. The pulp at this stage will show substantially no change in the usual analytical constants excepting a slight reduction in cuprammonium viscosity, of the order of 1 or 2 centipoises, and a lower content of ether-extractive material.

The acetylation of the dehydrated pulp may then be carried out, for example, by the process described in the copending application of Lyle Sheldon et al., S. N. 70,372, filed March 23, 1936, which consists briefly of cooling the cellulose to 25° C., treating at that temperature with a mixture of 2.45 parts of 95% acetic anhydride and 0.026 part of sulfuric acid per part of cellulose, and completing the reaction by allowing a gradual rise in temperature to 42.5° C. The acetate may then be precipitated or converted to the

acetone-soluble form and further treated by methods known in the art.

*Example B*

- 5 Cellulose, such as that described in Example A, containing 1.75 times its weight of moisture, is mixed with 5 parts of acetic acid, and subjected to dehydration with the use of 12.5 parts of normal propyl acetate per part of cellulose as described in the above example excepting that the distillation is carried out at atmospheric pressure and the maximum temperature to which the cellulose is heated is below 105° C. After substantial removal of the moisture has been effected, 15 the acetylation and further treatment may be carried out as described in Example A.

We have thus disclosed a process for rendering cellulose readily and economically convertible to cellulose acetate by means of which the 20 manufacturing cost from conventional raw materials may be reduced and less expensive raw materials made available for conversion which have heretofore been unsuitable. The basic features of the said process consist in starting with 25 cellulose which is saturated with water, adding acetic acid to the cellulose, and volatilizing the moisture with the vapor of a volatile organic solvent, which in the liquid state is totally miscible with acetic acid and immiscible with water, under conditions as specified, which avoid shrinkage and degradation of the cellulose and effect an improvement in the reactivity and purity thereof.

Cellulose which has been treated by the process of this invention is obtained in fluffy form, saturated with acetic acid, containing less than 2% moisture, and in a state of swelling substantially corresponding to that of its initial water-saturated condition. It is highly responsive to 30 treatment with acetylation mixtures, yielding useful cellulose acetate solutions at lowered cost. Acetic acid in the process may be replaced in whole or in part by the other low molecular weight fatty acids which are totally miscible with and less volatile than water, such as propionic and butyric acids. Such substitution is 35 particularly useful when the cellulose is to be converted to the propionate or butyrate, or mixed esters. Formic acid while a low molecular weight fatty acid totally miscible with water, is not uniformly less volatile than water and is not suitable for use in the process of this invention (International Critical Tables, vol. III, pages 212 and 215).

As many changes could be made in carrying out the above compositions and processes without departing from the scope of the invention, it is intended that all matter contained in the above description or shown in the accompanying drawing shall be interpreted as illustrative and not in a limiting sense.

In the foregoing specification and following claims, terms have been used having the following meanings:

**Alpha cellulose** is defined as that portion of a sample of cellulosic material not dissolved by 17.5% sodium hydroxide solution at 20° C., determined by a refinement of the method described by H. F. Lewis in "Technical Association Papers," 70 series XVII, #1436 (1934).

**Soda soluble material** is defined as that portion of a cellulosic sample dissolved when it is subjected to the action of 7.14% sodium hydroxide solution at the boiling point of water for 75 3 hours by a refinement of the method of Griffin,

"Technical Methods of Analysis," 492 (1927 ed.)

**Cuprammonium viscosity**, as used herein, means the viscosity number or value obtained according to the following method: The cuprammonium solution is prepared by the action of air on electrolytic copper in the presence of strong ammonia water. The copper concentration of the solutions employed for viscosity determinations is 30,  $\pm 2$  g. per liter and the ammonia content is 165 g.,  $\pm 2$  g. per liter. The concentration of cellulose employed is 0.6 g. (oven dry basis) per 100 cc. of cuprammonium solution. The cellulose sample for this determination is dried at 70° C. to 4% moisture content. After weighing out 0.6 g. (oven dry basis), the sample is moistened, squeezed to a weight of 2 g. and then dispersed in cuprammonium solution in an atmosphere of hydrogen from which oxygen has been completely removed. The viscosity measurements are made at 25° C. with a modified 20 Ostwald pipet, constructed according to the specifications of the Americal Chemical Society Committee on the Viscosity of Cellulose (Journal of Industrial & Engineering Chemistry, I, #49; 1929). The time of flow in seconds is converted 25 to centipoises on the basis of the calibration of the pipet with oils of known viscosity in centipoises obtained from the United States Bureau of Standards.

**Method for testing suitability of cellulose for acetylation.**—A 10 g. sample is agitated in 30 times its weight of water at room temperature for 15 minutes and then drained and pressed free of excess water. The operation is repeated four times using glacial acetic acid instead of water. 35 The drained and pressed cake finally obtained is weighed, placed in a suitable bottle in shredded condition, and brought to a temperature of 25° C. Sufficient glacial acetic acid, containing 0.36 g. of 96% sulfuric acid, is added to bring the total amount of acetic acid to 70 g. After thorough mixing and allowing the mixture to stand for 15 minutes at 25° C., 30 grams of acetic anhydride are incorporated into the mass and the mixture maintained at 40° C. for 30 minutes 45 with occasional stirring, when the reaction is stopped by adding 15 c. c. of 70% acetic acid. After entrapped air bubbles have been removed by applying suction and the mixture has been allowed to stand for 1 hour at 25° C., the color 50 and haze are measured and expressed in terms of the standards of the American Public Health Association described in "Standard Methods of Water Analysis," pp. 4-11 (1933 ed.). By the above procedure, a good quality of acetylable 55 cellulose will yield a reaction mixture having about 50 parts per million color and haze.

We claim:

1. The method of conditioning cellulose for chemical treatment comprising providing purified cellulose with its fibers in swollen condition and saturated with water, subjecting the said water-saturated cellulose to distillation in the presence of a low molecular weight fatty acid which is totally miscible with and uniformly less volatile than water such as acetic, propionic or butyric, and of an organic solvent which is miscible with and more volatile than the said acid and immiscible with water, said combined liquids forming a homogeneous liquid phase at distillation temperatures, and continuing the distillation until the cellulose is substantially free of water and solvent and saturated with said acid so as to maintain the cellulose fibers in swollen condition. 70
2. In the manufacture of a cellulose derivative 75

- including reaction with the cellulose in the presence of a low molecular weight fatty acid totally miscible with and uniformly less volatile than water such as acetic, propionic or butyric, the method of preparing cellulose for such reaction in swollen condition of its fibers substantially saturated with said acid and free from water which comprises providing water-swollen wood cellulose, and replacing the water with said acid while maintaining the cellulose fibers in swollen condition by subjecting the saturated cellulose in the presence of said acid to distillation of the water with an organic solvent which is immiscible with water, miscible with and more volatile than the said acid, and which forms an azeotropic mixture with the water having a boiling point below the temperatures at which cellulose is degraded, the acid, solvent, and water forming a homogeneous liquid phase, continuing said distillation to free said cellulose of said water and solvent and saturate said cellulose with acid in said swollen condition of the cellulose fibers, and then treating said cellulose to form said derivative.
3. In the manufacture of a cellulose derivative including reaction with cellulose in the presence of a low molecular weight fatty acid totally miscible with and uniformly less volatile than water such as acetic, propionic or butyric, the method of preparing cellulose for such reaction in swollen condition substantially saturated with said acid and free from water which comprises providing water-swollen wood cellulose and replacing the water in the cellulose with said acid while maintaining the cellulose in swollen condition, by subjecting the water-saturated cellulose to distillation in the presence of said acid with an organic solvent which is immiscible with water, miscible with said acid, and has a normal boiling point between 75° C. and 105° C., the acid, solvent, and water forming a homogeneous liquid phase continuing said distillation to free said cellulose of said water and solvent and saturate said cellulose with acid in said swollen condition of the cellulose fibers, and then treating said cellulose to form said derivative.
4. In the manufacture of cellulose acetate the method of preparing cellulose in swollen condition substantially saturated with acetic acid and free from water which comprises providing purified cellulose maintained in swollen condition by saturation with water, and replacing the water with acetic acid while maintaining the cellulose in swollen condition by subjecting the saturated cellulose and acetic acid to distillation with a volatile organic solvent which is immiscible with

water and miscible with acetic acid, has a normal boiling point between 75° C. and 105° C., and forms a homogeneous liquid phase with the water and acetic acid continuing said distillation to free said cellulose of said water and solvent and saturate said cellulose with said acid in said swollen condition of the cellulose fibers, and then treating said cellulose to form said acetate.

5. In the manufacture of cellulose acetate, the method of preparing cellulose in swollen condition substantially saturated with acetic acid and free from water which comprises providing cellulose maintained in swollen condition by saturation with water, and replacing the water with acetic acid while maintaining the cellulose in swollen condition by subjecting the saturated cellulose in the presence of acetic acid to distillation with an organic solvent of the group consisting of benzene, propyl acetate, isopropyl acetate and isopropyl ether, or mixtures of any of them, the said solvent forming with the acetic acid and water a homogeneous liquid phase, continuing said distillation to free said cellulose of said water and solvent and saturate said cellulose with said acid in said swollen condition of the cellulose fibers, and then treating said cellulose to form said acetate.

6. In the manufacture of cellulose acetate the process of preparing cellulose for acetylation which comprises removing water from the cellulose in the presence of acetic acid by distillation with a volatile organic solvent immiscible with water, miscible with acetic acid, and having a boiling point below that of acetic acid, subjecting the vapors to fractional condensation, and extracting soluble impurities from the cellulose by percolating the reflux liquid through the cellulose.

7. The method of conditioning cellulose for chemical treatment comprising providing cellulose saturated with water, subjecting said cellulose to distillation in the presence of a low molecular weight fatty acid which is totally miscible with and uniformly less volatile than water such as acetic, propionic, or butyric and of an organic solvent which is completely miscible with and more volatile than said acid and immiscible with water, the combined liquid forming a homogeneous liquid phase, subjecting the liquids to fractional condensation and extracting soluble impurities from said cellulose by percolating the reflux liquid through said cellulose and continuing the distillation until the cellulose is substantially free of water and solvent.

JOSEPH FLEISCHER.

WILLIAM A. BAILEY, JR.